



US005547809A

**United States Patent** [19]**Defieuw et al.**[11] **Patent Number:** **5,547,809**[45] **Date of Patent:** **Aug. 20, 1996**

[54] **THERMAL TRANSFER IMAGING SYSTEM  
BASED ON THE HEAT TRANSFER OF A  
REDUCING AGENT FOR REDUCING A  
SILVER SOURCE TO METALLIC SILVER**

[75] Inventors: **Geert Defieuw**, Kessel-Lo; **Wilhelmus Janssens**, Aarschot; **Luc Vanmaele**, Lochristi; **Jean-Marie Dewanckele**, Drongen; **Herman Uytterhoeven**, Bonheiden, all of Belgium

[73] Assignee: **Agfa-Gevaert, N.V.**, Mortsel, Belgium

[21] Appl. No.: **426,817**

[22] Filed: **Apr. 21, 1995**

[30] **Foreign Application Priority Data**

May 17, 1994 [EP] European Pat. Off. .... 94201382

[51] **Int. Cl.<sup>6</sup>** .... **G03C 8/08; G03C 8/24**

[52] **U.S. Cl.** .... **430/200; 430/203; 503/227**

[58] **Field of Search** .... 430/200, 203,  
430/201; 503/227

[56] **References Cited**

U.S. PATENT DOCUMENTS

3,094,417 6/1963 Workman .... 430/203  
3,218,166 11/1965 Reitter .... 430/203  
3,547,648 12/1970 Sagawa .... 430/203  
3,767,414 10/1973 Hoffman et al. .... 430/203  
3,795,532 3/1974 Newman et al. .... 430/620

3,941,596 3/1976 Heiart ..... 430/200  
4,013,473 3/1977 Willems et al. ..... 430/203  
5,310,640 5/1994 Markin et al. ..... 430/617  
5,322,833 6/1994 Defieuw et al. ..... 503/227  
5,374,514 12/1994 Kirk et al. ..... 430/619  
5,380,607 1/1995 Van Haute et al. ..... 430/200  
5,384,238 1/1995 Ellis et al. ..... 430/617

FOREIGN PATENT DOCUMENTS

246832 9/1960 Australia .  
2083726 3/1982 United Kingdom .

*Primary Examiner*—Richard L. Schilling  
*Attorney, Agent, or Firm*—Brumbaugh, Graves, Donohue & Raymond

[57] **ABSTRACT**

The present invention provides a printing process using a donor element and a receiving element. The donor element comprises on a support a donor layer comprising a binder and a thermotransferable strong reducing agent capable of reducing a silver source to metallic silver upon heating.

The donor element is image-wise heated while being in contact with an image receiving material comprising a thermoreducible silver source and a weak reducing agent, only being capable of reducing a silver source to metallic silver in the presence of metallic silver formed by said strong reducing agent. Image density is increased and stability of the reductor donor element can be improved.

**7 Claims, No Drawings**

**THERMAL TRANSFER IMAGING SYSTEM  
BASED ON THE HEAT TRANSFER OF A  
REDUCING AGENT FOR REDUCING A  
SILVER SOURCE TO METALLIC SILVER**

**DESCRIPTION**

**1. Field of the Invention**

The present invention relates to a thermal imaging process, more particular to a method wherein a thermotransferable strong reducing agent of a donor element is transferred image-wise to a receiving layer, comprising reducible silver source and a weak reducing agent.

**2. Background of the Invention**

Thermal imaging or thermography is a recording process wherein images are generated by the use of imagewise modulated thermal energy.

In thermography two approaches are known:

1. Direct thermal formation of a visible image pattern by imagewise heating of a recording material containing matter that by chemical or physical process changes colour or optical density.

2. Formation of a visible image pattern by transfer of a coloured species from an imagewise heated donor element onto a receptor element.

A survey of "direct thermal" imaging methods is given in the book "Imaging Systems" by Kurt I. Jacobson-Ralph E. Jacobson. The Focal Press—London and New York (1976), Chapter VII under the heading "7.1 Thermography". Thermography is concerned with materials which are not photosensitive, but are heat sensitive. Imagewise applied heat is sufficient to bring about a visible change in a thermosensitive imaging material.

According to a direct thermal embodiment operating by physical change, a recording material is used which contains a coloured support or support coated with a coloured layer which itself is overcoated with an opaque white light reflecting layer that can fuse to a clear, transparent state whereby the coloured support is no longer masked. Physical thermographic systems operating with such kind of recording material are described on pages 136 and 137 of the above mentioned book of Kurt I. Jacobson et al.

Thermal dye transfer printing is a recording method wherein a dye-donor element is used that is provided with a dye layer wherefrom dyed portions of incorporated dye is transferred onto a contacting receiving element by the application of heat in a pattern normally controlled by electronic information signals.

In thermal wax printing, the dye layer is transferred to the receiving element, whereas in thermal sublimation printing, also called dye diffusion thermal transfer (D2T2) only the dye is transferred to the receiving element. Thermal wax printing has problems to generate images with continuous tones, while the thermal sublimation printing technique offers only moderate densities (up to 2.5). It has been suggested to increase the density of a print made by thermal sublimation printing by printing several times on the same receiving sheet.

This procedure is slow and optical densities in transmission above 3.0 are hardly obtained with a good image stability. Another thermal imaging process described in European Patent Application nr. 94200612 and in European Patent Application nr. 94200794 uses (i) a reducto donor element comprising on a support a donor layer containing a binder and a thermotransferable reducing agent capable of reducing a silver source to metallic silver upon heating and

(ii) a receiving element comprising on a support a receiving layer comprising a silver source capable of being reduced by means of heat in the presence of a reducing agent, said thermal imaging process comprising the steps of

5 bringing said donor layer of said reducto donor element into face to face relationship with said receiving layer of said receiving element,

image-wise heating a thus obtained assemblage by means of a thermal head or a laser, thereby causing image-wise transfer of an amount of said thermotransferable reducing agent to said receiving element in accordance with the amount of heat supplied by said thermal head and

separating said donor element from said receiving element.

Prints obtained with both imaging processes mentioned above hardly obtain densities higher than 3.2–3.5. Moreover, a very high concentration of reducing agent is needed to obtain these high optical densities.

This leads to storage problems with the donor element (crystallisation and sticking in rolled form). It has been suggested to use mixtures of reducing agents in order to decrease the degree of crystallisation (such as mentioned in European Patent Application n° 94200795) or to decrease the degree of sticking of the donor element in rolled form by using particles in the donor layer (such as mentioned in European Patent Application n° 94200788). Donor elements yielding optical densities higher than 3.2–3.5 still suffer from these storage problems. These high optical densities are desired, especially for medical application.

**3. Object of the Present Invention**

It is an object of the present invention to provide a thermal imaging process wherein images are obtained with high optical densities, with a donor element having sufficient stability.

Further objects will become apparent from the description hereinafter.

According to the present invention, there is provided a thermal imaging process using (i) a donor element comprising on a support a donor layer containing a binder and a thermotransferable strong reducing agent capable of reducing a silver source to metallic silver and (ii) a receiving element comprising on a support a receiving layer comprising a weak reducing agent and a silver source capable of being reduced by means of heat in the presence of said strong reducing agent for said silver source, said thermal imaging process comprising the steps of

bringing said donor layer of said donor element into face to face relationship with said receiving layer of said receiving element,

image-wise heating a thus obtained assemblage thereby causing image-wise transfer of an amount of said strong thermotransferable reducing agent to said receiving element in accordance with the amount of heat supplied and

separating said donor element from said receiving element.

Image-wise heating in accordance with the present invention is preferably performed by means of a laser or a thermal head.

**4. Detailed Description of the Invention**

The terms weak and strong reducing agent in accordance with the present invention have the following meaning.

A strong reducing agent is an agent that is capable of reducing a silver ion to metallic silver by the application of heat while a weak reducing is only capable of doing so when

nuclei of metallic silver are present. A simple method to determine whether a reducing agent is weak or strong, is to coat a layer having the following composition:

|                               |                       |
|-------------------------------|-----------------------|
| compound I (see below)        | 0.34 g/m <sup>2</sup> |
|                               | (I)                   |
| polyvinylbutyral (Butval B79) | 4.5 g/m <sup>2</sup>  |
| silver behenate               | 4.5 g/m <sup>2</sup>  |
| reducing agent to test        | 2 g/m <sup>2</sup>    |

on a 175  $\mu\text{m}$  thick clear polyethylene terephthalate support. The obtained element is then heated from the back side on an aluminium hot plate at a temperature of 118 °C. for 10 seconds. A strong reducing agent will yield a visual density in transmission (measured on a Macbeth TR 924 calibrated to zero using the support film) of 0.25 or more while a weak reducing agent will show a visual density of less than 0.25.

Both strong and weak reducing agents may be selected from the group of the conventional photographic developers as described by the Kendall-Pelz rule (The Theory of the Photographic Process—T. H. James p. 289–299—fourth edition), such as phenidone, hydroquinones and catechol provided that the reducing agent is thermotransferable.

Suitable weak reducing agents can also be found in the class of so called rubber or polymer antioxidantia e.g. sterically hindered substituted 2,2'- or 4,4'-methylenebisphenol compounds.

Examples of suitable reducing agents are aminohydroxycycloalkenone compounds, esters of amino reductones, N-hydroxyurea derivatives, hydrazones of aldehydes and ketones, phosphoramidophenols, phosphoramidoanilines, polyhydroxybenzenes, e.g. hydroquinone, t-butylhydroquinone, isopropylhydroquinone, and (2,5-dihydroxyphenyl)methylsulfone, dihydroxybenzene derivatives such as pyrocatechol, and pyrogallol derivatives such as 4-phenylpyrocatechol, t-butylcatechol, pyrogallol, or pyrogallol derivatives such as pyrogallol ethers or esters, dihydroxybenzoic acid, dihydroxybenzoic acid esters such as dihydroxybenzoic acid, methyl ester, ethyl ester, propyl ester, butyl ester and the like, gallic acid, gallic acid esters such as methyl gallate, ethyl gallate, propyl gallate and the like, gallic acid amides, sulphydroxamic acids, sulfonamidoanilines, 2-tetrazolylthiohydroquinones, e.g., 2-methyl-5-(1-phenyl-5-tetrazolylthio)hydroquinone, tetrahydroquinoxalinines, e.g. 1,2,3,4-tetrahydroquinoxaline, amidoximes, azines, hydroxamic acids, 5-pyrazolones, sulfonamidophenol reducing agents, 2-phenylindan-1,3-dione and the like, 1,4-dihydropyridines, such as 2,6-dimethoxy-3,5-dicarboxy-1,4-dihydropyridine, bisphenols, e.g., bis(2-hydroxy-3-t-butyl-5-methylphenyl) methane, bis(6-hydroxy-m-tolyl)mesitol, 2,2-bis (4-hydroxy-3-methylphenyl)propane, 4,4-ethylened-bis(2-t-butyl-6-methylphenol) and 2,2-bis(3,5-dimethyl-4-hydroxyphenyl) propane, ascorbic acid derivatives and 3-pyrazolidones.

Reducing agents having a coloured oxidation product or wherein the oxidation product is capable of forming colour can also be used. Examples are 4-methoxynaphthol and leucoazomethines such as mentioned in European Patent Application n° 94200613.

The above mentioned method, to determine whether one of the described reducing agents is strong or weak, is used to evaluate if the reducing agent is advantageously added to the donor or the receiving element.

The donor element for use according to the present invention comprises on one side of the donor element a donor layer, comprising a strong reducing agent capable of reducing a silver source to metallic silver upon heating, and a binder.

Strong reducing agents selected from the group of pyrocatechol, pyrocatechol derivatives, gallic and gallolderivatives and leucoazomethines are preferred. Especially preferred strong reducing agents are 4-phenylpyrocatechol, gallic acid alkyl esters and dihydrobenzoic acid alkyl esters.

Two or more reducing agents can be used in the donor layer, provided at least one reducing agent is strong. It may be advantageous to use a thermotransferable dye in combination with said strong reducing agent. This is especially useful when black images having a neutral grey tone are required, e.g. in medical applications. The principle of the use of thermotransferable dyes is explained in more detail in European Patent Application n° 94200796.

As a binder for the donor layer, hydrophilic or hydrophobic binders can be used, although the use of hydrophobic binders is preferred.

Hydrophilic binders that can be used are polyvinylalcohol, gelatine, polyacrylamide and hydrophilic cellulosic binders such as hydroxyethyl cellulose, hydroxypropyl cellulose and the like.

The hydrophobic binders may be used as a dispersion in e.g. water or as a solution in an organic solvent.

Suitable binders for the donor layer are cellulose derivatives, such as ethyl cellulose, methyl cellulose, cellulose nitrate, cellulose acetate formate, cellulose acetate hydrogen phthalate, cellulose acetate, cellulose acetate propionate, cellulose acetate butyrate, cellulose acetate pentanoate, cellulose acetate benzoate, cellulose triacetate; vinyl-type resins and derivatives, such as polyvinyl acetate, polyvinyl butyral, copolyvinyl butyral-vinyl acetal-vinyl alcohol, polyvinyl pyrrolidone, polyvinyl acetoacetal, polyacrylamide; polymers and copolymers derived from acrylates and acrylate derivatives, such as polymethyl methacrylate and styreneacrylate copolymers; polyester resins; polycarbonates; copoly(styrene-co-acrylonitrile); polysulfones; polyphenylene oxide; organosilicones, such as polysiloxanes; epoxy resins and natural resins, such as gum arabic. Preferably, the binder for the donor layer of the present invention comprises poly(styrene-co-acrylonitrile).

The binder for the donor layer preferably comprises a copolymer comprising styrene units and acrylonitrile units, preferentially at least 60% by weight of styrene units and at least 25% by weight of acrylonitrile units binder. The binder copolymer may, of course, comprise other comonomers than styrene units and acrylonitrile units. Suitable other comonomers are e.g. butadiene, butyl acrylate, and methyl methacrylate. The binder copolymer preferably has a glass transition temperature of at least 50 °C.

It is, of course, possible to use a mixture of the copolymer comprising styrene units and at least 15% by weight of acrylonitrile units with another binder known in the art, but preferably the acrylonitrile copolymer is present in an amount of at least 50% by weight of the total amount of binder.

The donor layer generally has a thickness of about 0.2 to 5.0  $\mu\text{m}$ , preferably 0.4 to 2.0  $\mu\text{m}$ , and the amount ratio of reducing agent to binder generally ranges from 9:1 to 1:10 weight, preferably from 3:1 to 1:5 by weight.

The donor layer may also contain other additives such as i.a. thermal solvents, stabilizers, curing agents, preservatives, dispersing agents, antistatic agents, defoaming agents, and viscosity-controlling agents.

The donor layer may also contain particles protruding from the surface of the donor element, such as described in European Patent Application n° 94200788.

Highly preferred particles for use in connection with the present invention are polymethylsilsesquioxane particles such as e.g. Tospearl 120, Tospearl 130 and Tospearl 145 (Toshiba Silicone). In case a laser is used to heat the donor layer of the donor element, an infra-red absorbing substance is advantageously added to one of the layers of the donor element, preferably to the donor layer.

Any material can be used as the support for the donor element provided it is dimensionally stable and capable of withstanding the temperatures involved. Such materials include polyesters such as polyethylene terephthalate, polyamides, polyacrylates, polycarbonates, cellulose esters, fluorinated polymers, polyethers, polyacetals, polyolefins, polyimides, glassine paper and condenser paper. Preference is given to a support comprising polyethylene terephthalate. In general, suitable supports for use in combination with a thermal head can have a thickness of 2 to 30  $\mu\text{m}$ , preferably a thickness of 4 to 10  $\mu\text{m}$  is used. The thickness of the support for image-wise heating with a laser is less critical. Usually a thicker support of 30 to 300  $\mu\text{m}$  is used. The support may also be coated with an adhesive of subbing layer, if desired.

Subbing layers comprising aromatic copolymers, vinylidene chloride copolymers, organic titanate, zirconates and silanes, polyester urethanes and the like can be used.

The donor layer of the donor element can be coated on the support or printed thereon by a printing technique such as a gravure process.

A barrier layer comprising a hydrophilic polymer may also be employed between the support and the donor layer of the donor element to enhance the transfer of reducing agent by preventing wrong-way transfer of reducing agent backwards to the support. The barrier layer may contain any hydrophilic material that is useful for the intended purpose. In general, good results can be obtained with gelatin, polyacrylamide, polyisopropyl acrylamide, butyl methacrylate-grafted gelatin, ethyl methacrylate-grafted gelatin, ethyl acrylate-grafted gelatin, cellulose monoacetate, methylcelulose, polyvinyl alcohol, polyethyleneimine, polyacrylic acid, a mixture of polyvinyl alcohol and polyvinyl acetate, a mixture of polyvinyl alcohol and polyacrylic acid, or a mixture of cellulose monoacetate and polyacrylic acid.

Certain hydrophilic polymers e.g. those described in EP 227,091 also have an adequate adhesion to the support and the layer, so that the need for a separate adhesive or subbing layer is avoided. These particular hydrophilic polymers used in a single layer in the donor element thus perform a dual function, hence are referred to as barrier/subbing layers. The back side of the donor element for image-wise heating with a laser is not critical. Typically a transparent coating is used, incorporating particles to enhance the transport properties.

Owing to the fact that the thin support softens when heated by a thermal head during the printing operation and then sticks to the thermal printing head, thereby causing malfunction of the printing apparatus and reduction in image quality, the back of the support (the side opposite to that carrying the donor layer) is preferably provided with a heat-resistant layer to facilitate passage of the donor element past the thermal printing head. An adhesive layer may be provided between the support and the heat-resistant layer.

Any heat-resistant layers known in the field of thermal sublimation printing or wax printing can be used in the present invention.

The heat-resistant layer generally comprises a lubricant and a binder. In the conventional heat-resistant layers the

binder is either a cured binder as described in e.g. EP 153,880, EP 194,106, EP 314,348, EP 329,117, JP 60/151, 096, JP 60/229,787, JP 60/229,792, JP 60/229,795, JP 62/48, 589, JP 62/212,192, JP 62/259,889, JP 01/5884, JP 01/56, 587, and JP 92/128,899 or a polymeric thermoplast as described in e.g. EP 267,469, JP 58/187,396, JP 63/191,678, JP 63/191,679, JP 01/234,292, and JP 02/70,485.

During printing, a smooth transport of the donor ribbon and the receiving element is required in order to obtain a good density uniformity all over the print.

It is preferred to use different types of lubricants to allow continuous transport of the donor ribbon relative to the thermal head.

Well known lubricants are polysiloxanes such as those mentioned in EP 267,469, U.S. Pat. No. 4,738,950, U.S. Pat. No. 4,866,028, U.S. Pat. No. 4,753,920 and U.S. Pat. No. 4,782,041. Especially useful slipping agents are polysiloxane-polyether block or graft polymers.

Other lubricants for the heat-resistant slipping layer of the reductor donor element are phosphoric acid derivatives such as those mentioned in EP 153,880 and EP 194,106, metal salts of long fatty acids (such as mentioned in EP 458,538, EP 458,522, EP 314,348, JP 01/241,491 and JN 01/222,993), wax compounds such as polyolefin waxes such as e.g. polyethylene or polypropylene wax, carnauba wax, bees wax, glycerine monostearate, amid wax such as ethylene bisstearamide and the like.

A heat-resistant layer such as mentioned in European Patent Application no. 93 202 050.6 is especially preferred.

Inorganic particles such as salts derived from silica such as e.g. talc, clay, china clay, mica, chlorite, silica, or carbonates such as calcium carbonate, magnesium carbonate or calcium magnesium carboante (dolomite) can be further added to the heat-resistant layer.

It is highly preferred to add mixtures of particles to the heat resistant layer having a Mohs hardness below 2.7 and particles having a Mohs hardness above, 2.7 such as mentioned in EP-A-93201642.1.

A mixture of talc and dolomite particles is highly preferred.

A particular heat-resistant layer for the present invention comprises as a binder a polycarbonate derived from a bis-(hydroxyphenyl)-cycloalkane, corresponding to general formula (II):



wherein:

$\text{R}^1$ ,  $\text{R}^2$ ,  $\text{R}^3$ , and  $\text{R}^4$  each independently represents hydrogen halogen, a  $\text{C}_1\text{-C}_8$  alkyl group, a substituted  $\text{C}_1\text{-C}_8$  alkyl group, a  $\text{C}_5\text{-C}_6$  cycloalkyl group, a substituted  $\text{C}_5\text{-C}_6$  cycloalkyl group, a  $\text{C}_6\text{-C}_{10}$  aryl group, a substituted  $\text{C}_6\text{-C}_{10}$  aryl group, a  $\text{C}_7\text{-C}_{12}$  aralkyl group, or a substituted  $\text{C}_7\text{-C}_{12}$  aralkyl group; and

$\text{X}$  represents the atoms necessary to complete a 5- to 8-membered alicyclic ring, optionally substituted with a  $\text{C}_1\text{-C}_6$  alkyl group, a 5- or 6-membered cycloalkyl group or a fused-on 5- or 6-membered cycloalkyl group, as lubricants polyether modified polysiloxane block copolymer and zinc stearate and as particles talc particles with a mean size of 4.5  $\mu\text{m}$ .

Lubricants and binder can be coated in a single layer, or can be casted in a separate layer. It is highly preferred to cast

the salt of a fatty acid in the heat resistant layer (e.g. as a dispersion) and the polysiloxane based lubricant in a separate topcoat. This separate topcoat is preferably casted from a non-solvent for the heat-resistant layer.

The heat-resistant layer of the donor element may be coated on the support or printed thereon by a printing technique such as a gravure printing.

The heat-resistant layer thus formed has a thickness of about 0.1 to 3  $\mu\text{m}$ , preferably 0.3 to 1.5  $\mu\text{m}$ .

Preferably a subbing layer is provided between the support and the heat-resistant layer to promote the adhesion between the support and the heat-resistant layer. As subbing layer any of the subbing layers known in the art for dye-donor elements can be used. Suitable binders that can be used for the subbing layer can be chosen from the classes of polyester resins, polyurethane resins, polyester urethane resins, modified dextrans, modified cellulose, and copolymers comprising recurring units such as i.a. vinyl chloride, vinylidene chloride, vinyl acetate, acrylonitrile, methacrylate, acrylate, butadiene, and styrene (e.g. poly(vinylidene chloride)-co-acrylonitrile). Suitable subbing layers have been described in e.g. EP 138,483, EP 227,090, European Patent Application N) 92200907.1, U.S. Pat. No. 4,567,113, U.S. Pat. No. 4,572,860, U.S. Pat. No. 4,717,711, U.S. Pat. No. 4,559,273, U.S. Pat. No. 4,695,288, U.S. Pat. No. 4,727,057, U.S. Pat. No. 4,737,486, U.S. Pat. No. 4,965,239, U.S. Pat. No. 4,753,921, U.S. Pat. No. 4,895,830, U.S. Pat. No. 4,929,592, U.S. Pat. No. 4,748,150, U.S. Pat. No. 4,965,238, and U.S. Pat. No. 4,965,241.

The receiving element for use according to the printing method of the present invention comprises a receiving layer provided on a support, said receiving layer comprising a weak reducing agent and a silver source capable of being reduced by means of heat in the presence of a strong reducing agent. The way how a weak reducing agent can be selected has already been mentioned above.

Preferred weak reducing agents are selected from the group of sterically hindered phenols and sterically hindered bisphenols.

Usefull weak reducing agents are e.g.



50  
55  
60  
65

Compounds (V) and (VIII) are especially preferred. A mixture of weak reducing agents in the image receiving layer is particularly advantageous with regard to avoiding crystallisation during storage.

The reducible silver source may comprise any material that contains a reducible source of silver ions. Silver salts of organic and hetero-organic acids, particularly long chain fatty carboxylic acids (comprising from 10 to 30, preferably 15 to 25 carbon atoms) are preferred. Complexes of organic or inorganic silver salts in which the ligand has a gross stability constant for silver ion of between 4.0 and 10.0 are also useful. Examples of suitable silver salts are disclosed in Research Disclosure Nos. 17029 and 29963 and include: salts of organic acids, e.g., gallic acid, oxalic acid, behenic acid, stearic acid, palmitic acid, lauric acid and the like; silver carboxyalkylthiourea salts, e.g., 1-(3-carboxypropyl)thiourea, 1-(3-carboxypropyl)-3,3-dimethylthiourea and the like; complexes of silver with the polymeric reaction product of an aldehyde with a hydroxy-substituted aromatic carboxylic acid, e.g., aldehydes, such as formaldehyde, acetaldehyde and butyraldehyde, and hydroxy-substituted acids, such as salicylic acid, benilic acid, 3,5-dihydroxybenilic acid and 5,5-thiodisalicylic acid; silver salts or complexes of thiones, e.g., 3-(2-carboxyethyl)-4-hydroxymethyl-4-thiazoline-2-thione and 3-carboxymethyl-4-methyl-4-thiazoline-2-thione; complexes of salts of silver with nitrogen acids selected from imidazole, pyrazole, urazole, 1,2,4-triazole and 1H-tetrazole, 3-amino-5-benzylthio-1,2,4-triazole and benzotriazole; silver salts of saccharin, 5-chlorosalicylaldoxime and the like; and silver salts of mercaptides.

The preferred silver source is silver behenate.

The silver source is preferably added as a dispersion to the coating liquid of the receiving layer.

As binding agent for the heat sensitive layer preferably thermoplastic water insoluble resins are used wherein the

8  
-continued

(V)



(VI)



(VII)



(VIII)



ingredients can be dispersed homogeneously or form there with a solid-state solution. For that purpose all kinds of natural, modified natural or synthetic resins may be used, e.g. cellulose derivatives such as ethylcellulose, cellulose esters, carboxymethylcellulose, starch ethers, polymers derived from  $\alpha, \beta$ -ethenically unsaturated compounds such as polyvinyl chloride, after chlorinated polyvinyl chloride, copolymers of vinyl chloride and vinylidene chloride, copolymers of vinyl chloride and vinyl acetate, polyvinyl acetate and partially hydrolyzed polyvinyl acetate, polyvinyl alcohol, polyvinyl acetals, e.g. polyvinyl butyral, copolymers of acrylonitrile and acrylamide, polyacrylic acid esters, polymethacrylic acid esters and polyethylene or mixtures thereof. A particularly suitable ecologically interesting (halogen-free) binder is polyvinyl butyral. A polyvinyl butyral containing some vinyl alcohol units is marketed under the trade name BUTVAR B79 of Monsanto USA. Another interesting binder is cellulose acetate butyrate.

The binder to organic silver salt weight ratio is preferably in the range of 0.2 to 6, and the thickness of the image forming layer is preferably in the range of 5 to 16  $\mu\text{m}$ .

It is preferred to use a so-called toning agent in the receiving layer or in a layer adjacent to said receiving layer. This toning agent serves to change the tone of the silver image from brown to black or grey. Suitable toning agents are e.g. phthalazinone, phthalazine, phthalimide, succinimide, phthalic acid, benzimidazole or compound (I) as mentioned above.

The use of phthalazinone or compound (I) is highly preferred.

It is highly preferred to use a release agent on the receiving element on the side of the receiving layer. This release agent may be added to the coating solution of the receiving layer or may be applied, optionally in a mixture with other ingredients, as a separate layer called the release layer on top of said receiving layer. The use of a release layer is preferred, since the release agent is in that case on top of the receiving element.

The release agent is preferred in the printing method of the present invention since the reducing agents useful in the present invention may give rise to a sticky contact between donor element and receiving element.

As release agents, inorganic and organic release agents can be used. Among them, the organic release agent, are preferred.

Solid waxes, fluorine- or phosphate-containing surfactants and silicone oils can be used as releasing agent. Suitable releasing agents have been described in e.g. EP 133012, JP 85/19138, and EP 227092.

When, as mentioned above, a separate release layer, incorporating the release agent, is casted on top of said receiving layer, other ingredients such as binders, plasticizers, or particulate fillers such as talc, silica or colloidal particles can be added to said release layer, provided that the transfer of the reducing agent to the receiving layer comprising the reducible silver source can take place.

Examples of binders for the release layer are gelatin dextrans polyvinylbutyral, ethylcellulose, cellulose acetate propionate, cellulose acetate butyrate, polyvinylchloride, copolymers of vinylchloride, vinylacetate and vinylalcohol, aromatic or aliphatic copolymers, polymethylmethacrylate, polycarbonates derived from bisphenol A, polycarbonates comprising bisphenols according to formula (II) and the like. The release layer can also act as a protective layer for the images. Especially preferred release layers are mixtures of polyvinylbutyral with a silicon compound such as Tegoglide 410 or, mixtures of ethylcellulose with a silicon

compound or mixtures of a copolymer of poly(vinylchloride vinylacetate vinylalcohol), a difunctional polydimethylsiloxane such as Tegomer HSI 2111 and a di- or multifunctional isocyanate such as Desmodur VL or Desmodur N75.

An adhesive layer is usually provided between the support and the receiving layer, such as those mentioned in e.g. U.S. Pat. No. 4,748,150, U.S. Pat. No. 4,954,241, U.S. Pat. No. 4,965,239 and U.S. Pat. No. 4,965,238 and European Patent Application no. 92 201 620.9.

The subbing layer can further comprise other polymers, particles, or low molecular weight additives. Addition of inorganic particles such as silica, colloidal silica, water soluble polymers such as gelatin, polymeric latices, polystyrene sulfonic acid and polystyrene sulfonic acid sodium salt, surfactants such as cationic, anionic, amphoteric and non-ionic surfactants, and polymeric dispersants is preferred.

Especially preferred additives are colloidal silica, the above mentioned surfactants, butadiene containing latices such as poly(butadiene-co-methylmethacrylate-co-itaconic acid), polystyrene sulfonic acid and polystyrene sulfonic acid sodium salt. The addition of silica to the subbing layer decreases sticking on the coating roll after coating of the subbing layer. The addition of polystyrene sulfonic acid or polystyrene sulfonic acid sodium salt to the subbing layer accelerates the recycling process.

The subbing layer of the present invention is applied directly to the support of the receiving element. The subbing layer can be applied by coextrusion or can be coated on the support. Coating from aqueous solution is preferred due to its simplicity and the possibility of adding other ingredients.

The receiving layer is usually hydrophobic in order to enhance the absorption of reducing agent into the receiving element. The polyester recycling procedure, however, uses a cleaning step wherein the film waste is immersed in an alkaline or acid soap solution in water. It is an object of this cleaning process to remove all layers casted on the polymeric substrate.

In order to remove the hydrophobic receiving layer, it is highly preferred to cast an intermediate layer of an hydrophilic polymer between the subbing layer and the dye-receiving layer. This intermediate layer accelerates the cleaning step in the recycling procedure. Typical examples of hydrophilic polymers which can be used in such intermediate layers are polyvinyl alcohol, polyacrylamide, hydroxyethylcellulose, gelatin, polystyrene sulfonic acid, polyethylene glycol, poly(meth)acrylic acid, poly(meth)acrylic acid, alkali metal salts of polyacrylic acid, crosslinked copolymers containing (meth)acrylic acid or alkali metal salts of (meth)acrylic acid, alkali metal salts of polystyrene sulfonic acid, dextran, carrageenan and the like.

Anti-static coatings such as those described in EP 440,957 can be incorporated in the intermediate layer. This results both in a higher hydrophilicity and in better anti-static properties.

The intermediate layer may further comprise polymeric dispersions or latices, surfactants, inorganic particles such as silica and colloidal silica and the like. Addition of surfactants, colloidal silica and/or latices is preferred. Addition of silica to the intermediate layer decreases sticking to the coating roll after coating. Addition of latices to the intermediate layer improves the addition and improves the removing step in the recycling process in case of acrylic acid or methacrylic acid type latices.

The intermediate layer may also have a cushioning property, such as mentioned in U.S. Pat. No. 4,734,397.

A highly preferred intermediate layer is based on polystyrene sulphonic acid, hydroxyethylcellulose and an anionic surfactant.

## 11

The support for the receiving element may be a transparent film of e.g. polyethylene terephthalate, a polyether sulfone, a polyimide, a cellulose ester, or a polyvinyl alcohol-co-acetal. The support may also be a reflective one such as baryta-coated paper, polyethylene-coated paper, or white polyester i.e. white-pigmented polyester. Blue-coloured polyethylene terephthalate film can also be used as a support.

Although the subbing layer is useful for application on polyethylene-coated paper, substrates based on polyester, transparent or reflective, are preferred. In this case, the subbing layer can be applied before, during or after the biaxial stretching procedure.

At the opposite side of the receiving element (opposite to the receiving layer), a backcoat can be provided, optionally in combination, with an appropriate subbing layer to improve the adhesion between the backcoat and the support.

Hydrophilic as well as hydrophobic backcoats can be used. Hydrophilic backcoats can be applied easily from water, while hydrophobic backcoats have the advantage that the backcoat performs well at all humidity levels.

Examples of hydrophilic backcoat layers are layers comprising polyvinylalcohol, polyethylene glycol, polyacrylamide, hydroxyethylcellulose, dextran and gelatin. The use of gelatin is highly preferred.

These hydrophilic backcoat layers may further comprise dispersions or latices of hydrophobic polymers, inorganic particles, surfactant and the like. The addition of these particles can be used in order to obtain a specific surface gloss, such as mentioned in European patent application no. 91 203 008.7. Especially preferred particles are silica and polymethylmethacrylate beads of 0.5 to 10  $\mu\text{m}$ . Antistatic treatment can also be provided to said backcoat layer.

Examples of hydrophobic backcoat layers are backcoat layers comprising addition polymers such as polymethylmethacrylate, polyvinylchloride and polycondensates such as polyesters, polycarbonates in combination with the above mentioned particles for the hydrophilic backcoat layers.

With hydrophobic backcoat layers, it can be useful to provide an intermediate hydrophilic layer between the subbing layer and the backcoat layer, such as those mentioned for use at the receiving side of the receiving element, in order to improve the removal of the backcoat layer in the recycling procedure.

The printing method of the present invention preferably uses a thermal head to selectively heat specific portions of the donor element in contact with a receiving element. The thermal head can be a thick or thin film thermal head although.

The use of a thin film thermal head is preferred, since this offers more opportunities to obtain appropriate gradation. The pressure applied to the thermal head is preferably between 120 and 400 g/cm heater line. A spatial resolution of 150 dpi or higher is preferred. The average printing power is calculated as the total amount of energy applied during one line time divided by the line time and by the surface area of the heat-generating elements.

Although a higher average printing power results in higher optical densities of the final image, it is preferred to use an average printing power below 10 W/mm<sup>2</sup>. At higher printing energies, deformation of the receiving layer and/or receiving sheet occurs.

The time needed for printing one single line with the thermal head, also called the line time, is preferably below 45 ms. Longer line times result in longer printing times and more deformation of the receiving sheet and/or receiving layer.

## 12

In order to increase the density of the final image after printing line-by-line with a thermal head, an overall heat treatment of the receiving element may be performed. This heat treatment can be e.g. done with an infrared source, a heated air stream or a hot plate but is preferably done by means of a heated roller.

It is believed that during the overall heat treatment, the transferred reducing agent can further react with the reducible silver source.

By selecting the appropriate diameter and speed of the heated roller, the heat treatment time for the overall heating can be adjusted. Moreover, the heated rollers can be used to uncurl the receiving sheet after printing.

The following examples illustrate the invention in more detail without, however, limiting the scope thereof.

## EXAMPLES

## Preparation of the donor elements

## \* Donor element A

Both sides of a 5.7  $\mu\text{m}$  thick polyethylene terephthalate support were coated with a subbing layer of a copolyester comprising ethylene glycol, adipic acid, neopentyl glycol, terephthalic acid, isophthalic acid, and glycerol.

The resulting subbing layer was covered with a solution in methyl ethyl ketone of 13% of a polycarbonate having the following structural formula (X):



wherein n represents the number of units to obtain a polycarbonate having a relative viscosity of 1.30 as measured in a 0.5% solution in dichloromethane, 0.5% of talc (Nippon Talc P3, Interorganica) and 0.5% of zinc stearate.

Finally, a top layer of polyether-modified polydimethylsiloxane (Tegoglide 410, Goldschmidt) was coated from a solution in isopropanol on the resulting heat-resistant polycarbonate layer.

The other side of the reductor donor element was provided with a reductor layer.

A mixture of 10 weight % binder (Luran 388S, BASF), 10 weight % of 4-phenylpyrocatechol and 0.5 weight % Tospearl 145 was applied at a wet thickness of 10  $\mu\text{m}$  by means of a wire bar. The resulting layer was dried by evaporation of the solvent.

## \* Donor element B

The preparation as mentioned above for donor element A was repeated, except that a mixture of 8 weight % 4-phenylpyrocatechol, 5 weight % of propylgallate and 2% of a cyan dye having a structural formula XI:



was used instead of 10 weight % of 4-phenylpyrocatechol.

#### Preparation of the receiving elements

A subbed polyethylene terephthalate support having a thickness of 175  $\mu\text{m}$  was coated in order to obtain the following receiving layer:

silver behenate 4.5  $\text{g}/\text{m}^2$

compound I mentioned above 0.34  $\text{g}/\text{m}^2$

polyvinylbutyral (Butvar B79, Monsanto) 4.5  $\text{g}/\text{m}^2$

weak reducing agent (type and amount in table I)

After drying, a release layer was coated from hexane comprising 0.03  $\text{g}/\text{m}^2$  Tegolide 410 (polyether-polysiloxane blockcopolymer from Goldschmidt). These receiving elements were used in the following printing examples.

#### Printing of the combination of donor and receiving elements

Printing was performed by contacting the donor layer of the donor element with the receiving layer of the receiving element, followed by heating by means of a thermal head. The thermal head was a thin film thermal head heated at an average printing power of 5 Watt/ $\text{mm}^2$  and a line time of 18 ms with a resolution of 300 dpi. The pressure applied between the thermal head and the rotating drum carrying the receiving and donor element was 160 g/cm heater line. After printing, the receiving element was separated from the donor element.

The printed image was a 16-step grey scale between data level 0 and 255 (8 bit). The data levels of the different steps were chosen equidistant with respect to the input data level in order to obtain the native sensitometry.

#### Overall heat treatment

All receiving elements were reheated on a hot plate of 118° C. for 10 seconds.

#### Measurement of the optical density of the prints

The optical maximal densities of the prints were measured after a visual filter in a Macbeth TR924 densitometer in the grey scale part corresponding to data level 255.

The results are listed in table I.

TABLE I

| Example  | Compound | Receiving element<br>weak reducing agent |  | Optical density (visual)<br>Donor element |      |
|----------|----------|------------------------------------------|--|-------------------------------------------|------|
|          |          | Amount ( $\text{g}/\text{m}^2$ )         |  | A                                         | B    |
| 1 (comp) | None     | —                                        |  | 2.06                                      | 3.12 |
| 2        | III      | 1.92                                     |  | 3.24                                      | 3.62 |
| 3        | III      | 3.84                                     |  | 2.81                                      | 3.41 |

TABLE I-continued

| Example | Compound | Receiving element<br>weak reducing agent |  | Optical density (visual)<br>Donor element |      |
|---------|----------|------------------------------------------|--|-------------------------------------------|------|
|         |          | Amount ( $\text{g}/\text{m}^2$ )         |  | A                                         | B    |
| 4       | IV       | 5.02                                     |  | 2.33                                      | 3.25 |
| 5       | V        | 3.85                                     |  | 3.81                                      | 3.76 |
| 6       | V        | 7.71                                     |  | 3.93                                      | 3.93 |
| 7       | VI       | 1.82                                     |  | 3.52                                      | 3.76 |
| 8       | VI       | 3.64                                     |  | 3.94                                      | 4.11 |

It is clear from table I that high optical densities (up to 4) can be obtained by the above printing method. Moreover, this can be achieved with a donor element comprising a moderate amount of reducing agent (donor element A). Visual inspection of the prints demonstrate that good grey tones are obtained, even at these high densities.

We claim:

1. A thermal imaging process using (i) a donor element comprising on a support a donor layer containing a binder and a thermotransferable strong reducing agent capable of reducing a silver source to metallic silver and (ii) a receiving element comprising on a support a receiving layer comprising a silver source, capable of being reduced by means of heat in the presence of a strong reducing agent, and a weak reducing agent for said silver source, said thermal imaging process comprising the steps of

bringing said donor layer of said donor element into face to face relationship with said receiving layer of said receiving element

image-wise heating a thus obtained assemblage, thereby causing image-wise transfer of an amount of said thermotransferable strong reducing agent to said receiving element in accordance with the amount of heat supplied

separating said donor element from said receiving element,

and after said image-wise heating, applying an overall heat treatment to said receiving element,

wherein said strong reducing agent is capable of reducing a silver ion to metallic silver by the application of heat, and

wherein said weak reducing agent is capable of reducing a silver ion to metallic silver only in the presence of metallic silver nuclei.

2. A thermal imaging process according to claim 1, wherein said weak reducing agent in said receiving layer is only capable of substantially reducing said silver source in the presence of said strong reducing agent.

3. A thermal imaging process according to claim 2, wherein said silver source is silver behenate.

4. A thermal imaging process according to claim 1 wherein said receiving layer of said receiving element containing said silver source further comprises a toning agent.

5. A thermal imaging process according to claim 1 wherein said strong reducing agent is selected from the group consisting of pyrocatechol, pyrocatechol derivatives, gallo and gallo derivatives or leucoazomethines or mixtures thereof.

6. A thermal imaging process according to claim 1 wherein said weak reducing agent is selected from the group of sterically hindered phenols or sterically hindered bisphenols.

7. A thermal imaging process according to claim 1 wherein said overall heating is performed by means of a heated roller.

\* \* \* \* \*